

1

3,014,794  
PRODUCING ALKYLATE OF REDUCED COPPER  
CORROSION

Norman R. Le Roy, Manhattan Beach, Calif., assignor to  
California Research Corporation, San Francisco, Calif.,  
a corporation of Delaware  
No Drawing. Filed Feb. 9, 1960, Ser. No. 7,526  
4 Claims. (Cl. 44—76)

This invention relates to improvements in the art of alkylating olefins with isoparaffins in the presence of a sulfuric acid catalyst. In particular, the invention is concerned with a method of reducing the copper strip corrosivity of alkylate produced by the sulfuric acid process.

Alkylation is widely practiced as a method of producing gasoline boiling range hydrocarbons from lower molecular weight hydrocarbons. In the sulfuric acid alkylation process an isoparaffin, such as isobutane, is condensed with a mono-olefin, such as butylene, in the liquid phase at temperatures of 0—100° F. and in the presence of sulfuric acid. The hydrocarbon phase, or whole alkylate, is separated from the acid, neutralized with caustic, water washed, and distilled to separate unreacted light hydrocarbons and heavy alkylate from the gasoline boiling range product alkylate. The alkylate so produced by condensing isobutane with butylene is particularly well suited for use as aviation gasoline or as a major constituent in blended aviation gasoline. Generally, the gasoline may comprise from 25% to 75% alkylate, by volume, depending on the grade of gasoline.

Aviation gasoline specifications as set out in ASTM D-910 require that the gasoline pass the copper strip corrosion test, as described in ASTM D-130-56. As applied to gasoline, the copper strip corrosion test involves immersing a polished copper strip in a given quantity of the gasoline and then heating the stock for two hours at 212° F. in a closed container. The copper strip is then removed, washed, and rated by comparing visually with the ASTM copper strip corrosion standards. As applied to aviation gasoline, the test is reported as passing if there is no more than slight discoloration (strip numbers 0, 1A, or 1B). The copper strip test is indicative of the corrosivity of the stock, and it is highly sensitive in the detection of minute quantities of corrosive impurities.

Where the aviation gasoline contains alkylate produced by the sulfuric acid process, difficulty is sometimes encountered in passing this test. This problem periodically arises even though there has been no immediately apparent change in the alkylation operating conditions or in the neutralization, water-washing, or distillation steps.

It is an object of this invention to produce an alkylate which does not appreciably discolor a copper strip immersed therein for two hours at 212° F. A further object of the invention is to provide a method of reducing the copper strip corrosivity of the alkylate.

I have discovered that the copper strip corrosivity of alkylate produced by the sulfuric acid process can be reduced or, in most instances, completely eliminated by adding to the alkylate a minute quantity of a lower alkyl mercaptan. Briefly, the invention comprises adding to the alkylate a minor amount of alkyl mercaptans having less than six carbon atoms to the molecule, to provide a mercaptan concentration in the alkylate of from about 0.1 p.p.m. to less than 3 p.p.m. by volume, sufficient to inhibit the copper strip discoloration. Generally, less than 2 p.p.m. of mercaptan is required. At the low concentrations used the quantity of mercaptan is not sufficient to impart a disagreeable odor or to affect adversely any of the other specifications of the alkylate or gasoline containing the alkylate. The mercaptan concentration should be held below about 4 p.p.m. if the stock is required to

2

pass the doctor test, which is commonly required of military aviation gasoline although not specified in ASTM D-910. Additionally, with mercaptan concentrations above 3 p.p.m., there is a tendency to form white deposits in the copper strip test.

The mercaptans which may be used in the method of this invention comprise lower alkyl mercaptans, having less than 6 carbon atoms to the molecule, i.e., methyl, ethyl, propyl, butyl, and amyl mercaptans. Propyl, butyl, and amyl mercaptans are preferred because of their favorable boiling points. Mixed mercaptans containing one to five carbon atoms to the molecule have also been employed to advantage. The mercaptans are added to the finished alkylate obtained by caustic washing the crude whole alkylate, water washing, and distilling. A typical process flow and distillation scheme is described in U.S. Patent No. 2,346,770 to P. Lobdell and G. L. Mateer. Obviously, the mercaptans could be added later after blending of the alkylate with other gasoline stocks to form the finished gasoline. However, it is preferred that all blending stocks be brought on specification prior to blending.

*Example I*

While alkylate produced by condensing isobutane and butylene in the presence of sulfuric acid at 40° F. was caustic washed, water washed, and distilled to recover a finished alkylate boiling between 115° F. and 335° F. A sample of the finished alkylate was subjected to the copper strip test as set out in ASTM D-130-56, described previously. To three identical samples of the same alkylate were added 0.5, 1, and 2 p.p.m. by volume of butyl mercaptan. The experimental results are presented in the following table:

|    | Untreated<br>Alkylate    | Butyl Mercaptan Concentration |             |             |
|----|--------------------------|-------------------------------|-------------|-------------|
|    |                          | 0.5<br>p.p.m.                 | 1<br>p.p.m. | 2<br>p.p.m. |
| 40 | Copper Strip Rating..... | 2A                            | 1A          | 1A          |

In the evaluation of the copper strip test results, a rating of 2A indicates moderate tarnishing, in this case a claret red appearance. A rating of 1A indicates a light orange color, almost the same as a freshly polished strip.

*Example II*

Finished alkylate, recovered from whole alkylate as in Example I, had a copper strip rating of 2B (lavender). Treatment with butyl mercaptan brought the alkylate on specification, as shown by the data presented in the following table:

|    | Untreated<br>Alkylate    | Butyl Mercaptan Concentration |             |          |
|----|--------------------------|-------------------------------|-------------|----------|
|    |                          | 1<br>p.p.m.                   | 2<br>p.p.m. | 3 p.p.m. |
| 60 | Copper Strip Rating..... | 2B                            | 1B          | 1A       |

65 The rating 1B (orange) is also reported as passing the test for aviation gasoline.

*Example III*

70 Another sample of finished alkylate, recovered from whole alkylate in the same manner as in Example I, had a copper strip rating of 2A. After the addition of 1 p.p.m.

by volume of isopropyl mercaptan the copper strip rating was 1A.

*Example IV*

One part per million by volume of mixed mercaptans, comprising C<sub>1</sub>-C<sub>5</sub> mercaptans, was added to caustic-washed water-washed, and distilled finished alkylate having a copper strip test rating of 2A. The treated alkylate had a copper strip rating of 1A. The treated alkylate was blended with an aromatic distillate, primarily toluene, to produce an aviation gasoline containing 75 percent by volume treated alkylate, which gasoline was doctor sweet and passed all specifications set out in ASTM D-910.

The addition of lower alkyl mercaptans is also effective in improving the copper strip test of alkylate initially having a copper strip test of 3 (brassy tarnish) or 4 (black). However, a test of 4 indicates such severe contamination of the alkylate that it should instead be redistilled or otherwise purified, as by further caustic and water washing.

What I claim is:

1. The method of producing alkylate of reduced copper corrosivity, said alkylate being prepared by reacting an olefin with an isoparaffin in the presence of a sulfuric acid catalyst, which comprises neutralizing and water-washing alkylate separated from the reaction mixture and then

treating the alkylate with a minor amount of a lower alkyl mercaptan to provide a mercaptan concentration in the alkylate of from about 0.1 p.p.m. to less than 3 p.p.m. by volume.

2. The method of claim 1 wherein the mercaptan added is butyl mercaptan.

3. The method of claim 1 wherein the mercaptan added is a mixture of C<sub>1</sub>-C<sub>5</sub> mercaptans.

4. An aviation gasoline comprising predominantly alkylate, which gasoline does not discolor a copper strip immersed therein for two hours at 212° F., prepared by adding a minor amount, in the range 0.1 to less than 3 p.p.m. by volume, of alkyl mercaptans having less than 6 carbon atoms to the molecule to a neutralized water-washed and distilled finished alkylate, produced by condensing isobutane with butylene in the presence of a sulfuric acid catalyst, and blending the alkylate with a gasoline boiling range distillate.

20 References Cited in the file of this patent

UNITED STATES PATENTS

|           |                |       |               |
|-----------|----------------|-------|---------------|
| 2,033,877 | Burk           | ----- | Mar. 10, 1936 |
| 2,222,122 | Schulze et al. | ----- | Nov. 19, 1940 |
| 2,880,255 | Davis et al.   | ----- | Mar. 31, 1959 |